

Sept. 30, 1930.

H. C. HARVEY ET AL

1,776,790

RESIN COATED PULP BOARD

Filed Aug. 4, 1928

FIG. 1.



FIG. 2.



WITNESS

*G. V. Rasmussen*

BY

INVENTORS  
HAROLD C. HARVEY  
HUBERT L. BECHER  
By *President* *Curran*  
ATTORNEYS

## UNITED STATES PATENT OFFICE

HAROLD C. HARVEY, OF EWING TOWNSHIP, MERCER COUNTY, AND HUBERT L. BECHER, OF HAMILTON TOWNSHIP, MERCER COUNTY, NEW JERSEY, ASSIGNEES TO THE AGASOTE MILLBOARD COMPANY, OF EWING TOWNSHIP, NEW JERSEY, A CORPORATION OF NEW JERSEY

## RESIN-COATED PULP BOARD

Application filed August 4, 1928. Serial No. 297,534.

Our invention relates to pulp board containing a non-fluxing binder and coated with artificial resin.

Pulp board is usually made by running paper pulp, wood pulp or the like into a mold and, by means of pressure or otherwise, removing the majority of the water, (see, for instance, patent to D. M. Sutherland, Jr., No. 1,272,566 dated July 16, 1918) and subsequently drying out the remainder of the water by the application of heat, preferably in a suitably constructed dryer. There is usually added to the pulp, prior to shaping it in the mold, a suitable binder, either a fluxing binder or a non-fluxing binder. Our invention relates to a pulp board having added thereto a non-fluxing binder, for instance, a metallic soap. Such a non-fluxing binder is described in the patent to Hubert L. Becher, No. 1,678,720, dated July 31, 1928. This patent describes the use, as a binder, of a soap prepared from drying oils, such as linseed oil or China-wood oil, or from rosin, which is precipitated after the conclusion of the beating operation by the addition of a precipitant, such as commercial sulfate of aluminum, to convert the soap (for instance sodium soap of linseed oil) into an insoluble soap (for instance, aluminum linoleate.) In such application there is described furthermore the use of tannic acid as a dispersing agent for the soap. Instead of tannic acid there may be used a small proportion of a material, for instance red gum (the natural resin obtained from the Xanthorrhoea tree) which substance, if present in large quantities, would constitute a fluxing binder but in the comparatively small quantity necessary to obtain the desired dispersion is negligible in its effect on such binder from the standpoint of our invention.

When pulp board containing a non-fluxing binder has been produced in the manner hereinabove described, namely, by first having the majority of the water removed by means of pressure or otherwise from the material as it comes from the mold, and the remainder then removed by the application of heat, it is a commercial article (except possibly for subsequent shaping operations, such

as coacting or bending, or subsequent surfacing operations such as sanding) such as has been known in the market for many years.

Upon a completed board of this type as a body layer we place one or more sheets of paper on other suitable fibrous material, impregnated with a phenolic or other artificial resin of the class which is transformed under pressure and high heat to a hard insoluble and infusible condition, for instance, unsized paper impregnated with a varnish or other solution of phenolic resin. In the preferred form of our invention, we place also one or more of such sheets (preferably at least three), similarly impregnated, below the board so as to coat both sides thereof. This aggregate of sheets and board we place between the hollow platens of a press of the well known type (shown, for instance, in patent to Sutherland, No. 1,506,509 dated August 26, 1924) and then subject such aggregate to sufficient heat and pressure to bring the resin into its final insoluble and infusible condition. Before releasing the pressure we permit the aggregate to cool, for instance, by flooding the platens with cold water so that any moisture which may be present in the board will not be able to form steam as the pressure is released and thus do damage to the board or resin coating. As the result of the application of heat and pressure the resin has not only been converted into its final form but has been caused to form with the sheets an aggregate which in turn has been caused to adhere firmly to the board.

The outermost layer of paper may, prior to the application of resin, be provided with a suitable design, for instance, wood graining, and this will be visible through the outermost resin layer and add to the artistic effect of the finished article. Although in accordance with our invention only one side of the board need be coated in the manner described, we prefer to coat both sides thereof so as to prevent a warping of the board which might be caused by the entrance of moisture, or by stresses set up in the resin layer on one side of the board which would have no counter-

balancing stresses on the other side of the board.

Our invention is based upon the discovery that a board of the type hereinabove described is sufficiently elastic to act as a cushion to compensate for any unevenness in the surface or surfaces of the platen or platens coming into contact with the resin. Any unevenness in the surface in contact with the resin, for instance, a departure of even 1/5000 of an inch of such surface from a true plane, would cause an unevenness of finish which would render the resulting product unsalable for any use in which the beauty of such product is important. By our process a satisfactorily uniform gloss may be produced.

It is obvious that the board must possess elasticity sufficient to effect the objects of our invention and should therefore be thicker than the surface layer which is to be applied thereto. While we do not know of any pulp board of the type described which is not sufficiently elastic to enable a plurality of resin-impregnated sheets of paper to be applied thereto with a resultant satisfactory gloss, we desire it to be understood that if such a board exists, or may hereafter be discovered, we do not intend to include it in the expression "pulp board with non-fluxing binder" used in our claim. The great practical advantage of our invention is that we can coat satisfactorily a comparatively hard pulp board with only two or three sheets of resin-impregnated paper, thus obtaining a beautiful product at a very low cost.

In the accompanying drawing illustrating our invention, Fig. 1 shows the board of fibre and non-fluxing binder and sheets of fibrous material such as paper, impregnated with resin, before compression, and Fig. 2 shows the same after compression, the legends applied to the drawings being self-explanatory and replacing the usual reference characters. The thickness of the paper sheets shown in the drawing, in proportion to the thickness of the board, is greatly exaggerated for the sake of clearness.

#### Example

50 1000 pounds of waste paper are beaten in a beater or other suitable mixing engine with from 110 to 130 pounds of a soap prepared from drying oils, such as linseed oil or China-wood oil, or rosin to which soap has been added from 10 to 20% of its weight of tannic acid, preferably in the form of a commercial tanning extract. When the beating operation has been completed, the soap is precipitated by the addition, for instance 45 to 55 pounds, of commercial sulfate of aluminum. The resulting mixture is run into a mold, for instance, such as described in patent to Sutherland, No. 1,272,566 dated July 16, 1918, from which a large proportion of the water is removed by suction or draining, so much

fibrous material being placed into the mold that the finished board has a thickness of about one-half an inch. The loosely molded pulp is then subjected to pressure in a suitable press for the removal of as much water as can suitably be removed by a pressing operation, and is then placed in a suitably constructed dryer, for instance, one of the well known Coe type. As this board has been made with the aid of a non-fluxing binder, it contains only a comparatively small amount of water when it enters the dryer so that the dried board is very compact, although the removal of the water has left it just sufficiently spongy or elastic to enable it to act as a cushion in the manner hereinabove described. To each side of the board are applied three sheets of paper, each sheet impregnated with a phenol formaldehyde resin of the type well known in commerce, in the manner well known in the art. The aggregate of board and sheets is then subjected between suitable platens to sufficient heat and pressure to convert the resin into the final insoluble and infusible state, such operation at the same time causing the resin coated papers to form with the board a firmly united product. Care should be taken to have the surfaces of the platens as smooth and nearly true planes as possible; if desired highly polished steel or copper plates may be placed between platen and resin.

In order to secure the strongest possible adhesion between the board and the resin coating, it is advantageous to impregnate the surface or surfaces of the board with a liquid artificial resin, for instance, by dipping the board into a varnish made of such resin and then gently heating it so as somewhat to set the resin without, however, bringing it over into the infusible stage. This resin coating will, after the board has been completed, adhere firmly to the board by interlocking with the surface fibres thereof and will adhere firmly also to the superimposed resin layer, thus causing a very firm adhesion between such resin layer and the board.

Instead of the paper, we may use any other suitable material in sheet form, such as cloth or felt, capable of absorbing fluid artificial resin. For instance, the outermost sheet may be constituted by a piece of cloth woven or printed in colored design; we may also have the same design printed on all the sheets, so that if the outer layer is worn through or otherwise damaged, the appearance of the next layer may be in harmony with the remainder of the outermost layer.

We claim:

An article of manufacture consisting of a body layer and a superposed surface layer, the body layer being of much greater thickness than the surface layer and consisting of a homogeneous pulp board impregnated sub-

stantially throughout with a non-fluxing binder, and the surface layer consisting of one or more sheets of fibrous material embedded in hardened artificial resin and having a uniform finish, said layers being permanently secured at their meeting faces by means of such resin.

**HAROLD C. HARVEY.  
HUBERT L. BECHER.**

10

15

20

25

30

35

40

45

50

55

60

65